

## UNITED STATES PATENT OFFICE

ALBERT C. FISCHER, OF CHICAGO, ILLINOIS, ASSIGNOR TO THE PHILIP CAREY MANUFACTURING COMPANY, A CORPORATION OF OHIO

## COMPOSITION CONSTRUCTIONAL UNIT

No Drawing.

Application filed May 5, 1926. Serial No. 103,984.

This invention relates to composition constructional units composed of a mixture of ductile waterproofing material and animal hair, these units comprising such articles as 5 expansion joint roofing, planking, siding, floor covering, rail filler, protection course for paving and the like.

Heretofore it has been customary to manufacture felts, running them thru a saturating 10 vat, pressing out the excess saturation and then coating the saturated felts with an asphalt coating, using a suitable mineral material to prevent adhesion in the process of rolling or packing.

15 Other methods followed have been to mix the fibres of the felt with the asphalt in a heated state and then roll to the proper thickness while in a heated plastic state. Felt fibres, as known in the roofing art, are ultimately fibres of cotton rags, linters etc., which have no extended binding strength.

Because of the heavier body structure of an expansion joint, and the fact that it must be made up in thicknesses from  $\frac{1}{4}$  to 1 inch, 25 and in lengths of 5 feet, which are standard up to 15 feet, and from 3 to 12 inches or more in width, it is exceedingly important that the expansion strip have sufficient tensile strength to withstand excess warpage and 30 handling, because the strip must be set on edge in the road to permit of plastic material being poured on either side. These facts are known in the art.

This invention relates more particularly to 35 an elastic compressible body of elongated fibres, especially animal fibres, which are coated and pressed into a felted sheet, adding much greater tensile strength thereto than the short fibres, and in this particular instance 40 alludes particularly to the strength of animal hair, together with its unpenetrable nature, its rounded form and adaptability to interlacing, thus extending thru a considerable mass of bituminous material and binding the material together over an extended area, and has 45 to do particularly with the process as described in the original case in its relation to the paragraph reciting the following:

Another purpose of this invention is to provide a material for the purposes described in

sheets with considerably longer fibres than is usually provided in soft felt roofing sheets and felts as heretofore manufactured, the fibres of the roofing sheets being very small and short. The fibres of the material used 55 in the present invention in some instances may be as long as 2 or 3 inches. Flax, hemp, sisal and other vegetable fibres are preferable, although other mineral or animal fibres may also be employed in mixing fibrous material with bituminous material. The art, as taught by me, is familiar with the fact that the mass cannot be formed in a sheet for expansion joint purposes unless the mass of bituminous material or binder is considerably 60 greater than the fibrous material, and proportions exceeding thirty per cent of fibrous matter are not desirable because of the interference with the binding of the mass, thus making the mass unsatisfactory for expansion 65 joint purposes. This fact distinguishes material for expansion joint requirements as against merely coated fibres, which are made in sheet form for the purpose of insulating, which under no condition answers the purpose 70 of expansion joint because insulation materials must have a large proportion of air cells, and consequently the bulk of the mass or mixture is largely fibrous material as against the 75 binding material.

80 Animal fibre is particularly resilient when mixed with a bulk of bituminous material or elastic binding material and relates particularly to thoroughly waterproofing the animal hair in the proper mixing contrivance and matted same together under pressure to effect a continuous sheet suitable for use as an expansion joint and distinguishes as against what is known as a bat of hair felt, known to the art, which is dense by reason 85 of its requirements being primarily for insulating purposes that it is undesirable as an expansion joint, would not be economical because of the tremendous cost of treated hair 90 felt, and because the larger volume of the mass is constituted of the hairlike fibres densely matted even in the dry state. This is 95 not the case in the use of animal hair as devised by me for expansion joints.

Powerful mixers are employed, in which heated asphalt is placed and the animal hair is thrown into the mixture in the proper proportions, thoroughly mixed, and the entire mass thus subjected to pressure, in which the fibrous material thus coated with bituminous binder is compressed and matted together by passing same thru suitable pressure rolls. This effects a very economical and effective 10 expansion joint because the animal hair exerts its influence in preventing an excess of rapid oozing of the bituminous binder under pressure, yet in practise the passing traffic, because of the preponderance of binder, would 15 press the material back into the crevice if any undue elongation occurred.

The distinguishing feature in this invention is the long filament of animal hair employed because of its peculiar functioning 20 and binding power, as distinguished over other vegetable or mineral fibres.

I claim:

1. A preformed compressible and expandible constructional unit comprising a normally 25 plastic strip of ductile waterproofing material having relatively long animal hairs incorporated and distributed therein to give an elastic character to the strip, and the proportion of waterproofing material preponderating.

2. A preformed compressible and expandible constructional unit comprising a normally plastic strip of ductile waterproofing material having animal hairs approximating 35 one, two or three inches in length incorporated and distributed therein to give an elastic character to the strip, the proportion of waterproofing material preponderating.

3. A preformed expansion joint comprising 40 a normally plastic strip of ductile bituminous material having relatively long, coarse animal hairs, incorporated and distributed therein to give an elastic character to the strip, the proportion of binder preponderating.

4. A preformed expansion joint comprising 45 a normally plastic strip of ductile bituminous material having relatively long, coarse animal hairs uniformly distributed therein to give an elastic character to the strip, the proportions of hair not exceeding substantially thirty per cent.

5. A preformed expansion joint comprising 55 a normally plastic strip of ductile bituminous material having relatively long, elastic, flexible animal fiber uniformly incorporated therein, the proportion of the elastic, flexible fiber not exceeding substantially thirty per cent.

6. A preformed compressible and expandible constructional unit comprising a preponderance of ductile bituminous material in 65 strip form, said ductile bituminous material having uniformly incorporated therein elas-

tic, flexible, animal fiber not exceeding thirty per cent.

Signed at Chicago, Illinois, this 20th day of April, 1926.

ALBERT C. FISCHER. 70

75

80

85

90

95

100

105

110

115

120

125

130